

(Model.)

J. B. HALBERT.  
Brush.

No. 240,410.

Patented April 19, 1881.

Fig. I.



Fig. II.



Attest

John S. Jones

Eugene L. Frinkous

Inventor

John B. Halbert,  
by Wood S. Bond,  
his Attorney &c.

# UNITED STATES PATENT OFFICE.

JOHN B. HALBERT, OF LONGWOOD, FLORIDA, ASSIGNOR OF ONE-HALF TO  
E. W. HENCK AND LEMUEL POPE, OF SAME PLACE; SAID HENCK AND  
POPE ASSIGNSORS OF ONE-FOURTH OF THEIR RIGHT TO GEO. B. HODGE,  
OF NEWPORT, KENTUCKY.

## BRUSH.

SPECIFICATION forming part of Letters Patent No. 240,410, dated April 19, 1881.

Application filed March 19, 1881. (Model.)

*To all whom it may concern:*

Be it known that I, JOHN B. HALBERT, a citizen of the United States, residing at Longwood, in the county of Orange and State of Florida, have invented or discovered a new and useful Improvement in the Art of Making Brushes, whereby I am enabled to produce a new and useful article of manufacture, of which the following is a specification.

10 In the accompanying drawings I have illustrated a brush constructed according to my invention.

Figure 1 is a perspective view, and Fig. 2 a longitudinal vertical sectional view.

15 I take the green palmetto-root, which is cut into the desired length and shape, out of which the brush is formed, with the grain of the root running vertical, so that the fibers thereof will form a material and answer the purpose of 20 bristles of a brush. The pith or fibrous portion of the roots is then removed by being hammered out at one end of the block to a greater or less distance, which leaves the fibrous portion A of the root projecting from the remaining portion, B, of the block of sufficient stiffness and thickly studded or set to form the 25 tuft of the brush. The stiffness of the tuft or bristle of projecting fibers forming the brush proper is determined by the length of the fiber- 30 projections. The greater the distance the pith is removed from the block the longer and softer will be the brush.

35 The fiber of the palmetto-root makes a superior, tough, elastic brush, and has superior merit over any material now in use.

The backing of the brush is formed of the root itself, and may be made of any desired shape or form and attached to any of the well-known brush-handles now in use.

The object of my invention is to make from 40 the palmetto-root brushes of all kinds and adapted to the various uses known to the art.

A brush has heretofore been constructed from the bark of bass-wood reduced to a fiber at one end, several pieces of such wood being bound 45 and held together by a ferrule, in which is fitted a handle; but a brush constructed in this manner does not possess the peculiar characteristics of a brush constructed according to my invention, and is not claimed by me. 50

What I claim as my invention is—

1. The process of making a brush from the palmetto root by cutting the same into blocks of the desired shape and removing the pith surrounding the fiber from one portion of the 55 block, so as to leave projecting fibers to form the tuft of the brush.

2. As a new article of manufacture, a brush made from a palmetto-root in which the pith is removed from the fiber in a portion of the 60 block, which fiber forms the tuft of the brush.

In testimony whereof I have hereunto set my hand in the presence of two subscribing witnesses.

JNO. B. HALBERT.

Witnesses:

EDGAR HARRISON,  
H. H. SCARLETT.